

March 23, 1943.

A. BRANDT

2,314,854

HEAT TREATMENT OF MAGNESIUM BASE ALLOYS

Original Filed Oct. 8, 1941



Inventor:

Alfred Brandt

By Pierce & Scheffler

his Attorneys.

## UNITED STATES PATENT OFFICE

2,314,854

HEAT TREATMENT OF MAGNESIUM  
BASE ALLOYS

Alfred Brandt, Swansea, Wales, assignor, by  
mesne assignments, to The Anglo California  
National Bank of San Francisco, San Francisco,  
Calif., a national banking association, as trustee

Original application October 8, 1941, Serial No.  
414,176. Divided and this application August  
5, 1942, Serial No. 453,731. In Great Britain  
September 9, 1940

2 Claims. (Cl. 148—21.3)

This invention relates to high percentage magnesium base alloys and is particularly concerned with raising the yield point (proof stress) of the alloys by subjecting the same in the "as-cast" condition to a single-step heat treatment within a range of not less than 100° C. but less than 250° C., having avoided any previous thermal treatment at higher temperatures.

It is an object of the present invention to avoid the so-called solution heat treatment at temperatures far above 250°, which constitutes, with subsequent chilling, the first stage of the thermal treatment of magnesium base alloys which has theretofore been the standard practice in treating castings of this type, an annealing treatment at a lower temperature, below 200° C., being preferably carried out as a second stage. The single-step thermal treatment at low temperature leaves the strength of the material substantially unaltered, and the elongation may even decrease to some extent. On the other hand, the yield point is materially increased. Uniformity of results, reduction of wastage, the lessening of fire risks, are also possible advantages.

According to the present invention, the single-step heat treatment between 100° C. and 250° C. is applied to magnesium base alloys containing more than 7% but less than 12% of aluminum, and also containing from 0.1% to 1.0% of manganese, the total amount of alloying constituents being not above 12%.

The following examples illustrate various instances which are according to the present invention, the percentages being by weight and subject to tolerances for usual impurities.

The drawing shows the results of tests with various magnesium base alloy castings indicating both the yield point, in tons per square inch, for 0.1% permanent deformation in the alloy in the cast and non-heat treated condition and in respect of the cast alloy heat treated to give what appear to be optimum results, the abscissae being arranged in order of decreasing amounts of total alloying constituents and ordinates corresponding to yield point in tons per square inch.

Turning now to Figure 1 and reading from the left, the effect of the heat treatment of magnesium base alloy castings A to C inclusive of the hereinafter occurring table is illustrated. The top line of each of the various columns in the drawing indicates the yield point in tons per square inch of the heat-treated casting, the line in the same column somewhat below it indicating

the yield point of the unheat-treated alloy, that is to say, the alloy in the condition resulting from casting, or in other words, the condition known as "as cast" condition.

5 The table given below contains the percentages by weight of the casting subject to tolerance for usual impurities together with the heat treatment which they received, namely:

| 10   | Al    | Mn   | Total | Heat treatment in days at °C. |
|------|-------|------|-------|-------------------------------|
| 15 A | 11.28 | 0.31 | 11.59 | 3 x 175                       |
| B    | 10.39 | 0.66 | 11.05 | 3 x 140                       |
| C    | 6.57  | 0.33 | 6.90  | 1 x 175                       |

20 In preparing the above examples and diagrams, alloys were made up and cast into tensile test bars in accordance with the specifications of the British Air Ministry Department of Technical Development. Yield point, in tons per square inch, for 0.1% permanent elongation was determined in the case of each alloy in the "as cast" condition, and after heat treatment at 140° C. for 1, 2 and 3 days, after heat treatment at 175° C. for 1, 2 and 3 days, after heat treatment at 240° C. for 1, 2 and 3 days. Duplicate tests were carried out in each case. This application is a division of my application Serial No. 414,176, filed October 8, 1941.

I claim:

35 1. A method for improving the yield point of cast magnesium base alloys containing more than 7% but less than 12% of aluminum and from 0.1% to 1.0% of manganese, the total amount of alloying constituents being not above 12% the balance being substantially all magnesium, which comprises subjecting such alloys in the "as-cast" condition to a heat treatment at a temperature within the range of 100° C. to 250° C.

40 2. An alloy consisting principally of magnesium and containing from 7 to 12% of aluminum and from 0.1% to 1.0% of manganese, and the balance substantially all magnesium, the total amount of alloying constituents not exceeding 12%, in the form of shaped castings the yield point of which has been raised without appreciable increase in strength by heat treatment in 45 the "as-cast" condition at a temperature within the range of 100° C. to 250° C.

ALFRED BRANDT.